

1

2,758,088

## PENETRATING OIL COMPOSITION

Jeffrey H. Bartlett, Westfield, Delmer L. Cottle, Highland Park, and Hugh C. De Hoff, Roselle Park, N. J., assignors to Esso Research and Engineering Company, a corporation of Delaware

No Drawing. Application December 30, 1953,  
Serial No. 401,438

8 Claims. (Cl. 252—45)

This invention relates to improved penetrating oils. Particularly, the invention relates to lubricating oil compositions having improved penetrating power. More particularly, the invention relates to lubricating oil compositions containing combined therein a minor, but penetrating power improving amount, of the acetals or thioacetals of alcohols or mercaptans.

In the manufacture of lubricating oils, process oils, metal working compositions, and cutting oils, it is frequently desirable to enhance their natural penetrating ability and the closely related ability to spread over a large surface. It has been found that unblended hydrocarbon oils and fatty oils differ considerably in this respect, even though they have substantially the same viscosity at the temperature of the test. It has been found also that the addition of certain materials to such oils, even in relatively small amounts, greatly increases their ability to spread over a wide area and to penetrate small crevices.

For instance, U. S. Patent 2,263,265, which issued November 18, 1941, discloses that esters of carbonic acid, whether short or long chain esters, are very effective and possess to a marked degree the property of improving the penetrating and spreading power of oils.

It has now been found, and forms the object of this invention, that the acetals and thio-acetals of alcohols or mercaptans, also have the ability to considerably enhance the natural penetrating power of lubricating oils.

The acetals and thio-acetals which have been found to possess this property of enhancing the penetrating power of lubricating oils are preferably the acetals and mercaptals of branched chain alcohols and aldehydes. For example, the acetals of the Oxo alcohols and acetals having from 4 to about 18 carbon atoms are especially desirable.

The materials contemplated for use in preparing the penetrating oils of this invention may be described by the following formula:



wherein R is an alkyl radical derived from an aldehyde and contains from 4 to 18 carbon atoms, R' is an alkyl radical derived from an alcohol or a mercaptan containing from 4 to 18 carbon atoms, and wherein X is oxygen or sulfur.

Among the compounds operable in preparing the acetals and thio-acetals that may be used to prepare the penetrating oils of the instant invention are the following:

| Alcohols                           | Aldehydes                         |
|------------------------------------|-----------------------------------|
| Butyl alcohol                      | Butyraldehyde                     |
| Octyl alcohol                      | Octaldehyde                       |
| Isooctyl alcohol                   | Isooctaldehyde                    |
| Decyl alcohol                      | Decaldehyde                       |
| Isodecyl alcohol                   | Isodecaldehyde                    |
| Tridecyl alcohol                   | Tridecaldehyde                    |
| Isotridecyl alcohol                | Isoisotridecaldehyde              |
| C <sub>8-13</sub> Oxo alcohols     | C <sub>8-13</sub> Oxo aldehydes   |
| C <sub>4-18</sub> Aldol alcohols   | C <sub>4-18</sub> Aldol aldehydes |
| C <sub>4-18</sub> Guerbet alcohols |                                   |

2

The corresponding mercaptans of the above alcohols may also be used. Especially preferred are the alcohols and aldehydes having from 8-13 carbon atoms each.

The compounds of this invention are quite simply made by process known to the art. An example of one method of preparation is as follows:

688 (4 mols) gm. of C<sub>10</sub> Oxo alcohol and 256 gms. (2 mols) C<sub>8</sub> Oxo aldehyde, 2 grams of toluene sulfonic acid and 300 cc. of benzol were charged to a 3 liter 4-necked flask equipped with a water trap, condenser, and a thermometer. The mixture was refluxed for 3½ hours during which time 36 cc. of water was collected. The resulting mixture was washed 2 times with 5% NaOH and 3 times with water, then dried with potassium carbonate. It was filtered, the benzol evaporated on a steam bath, and distilled in a short path still. At .3 mm. Hg 610 gms. of product was obtained boiling between 150 and 158° C.

20 Mercaptans may be substituted for the alcohols in the above detailed procedure.

The acetals and mercaptals described above may be blended in any of the commonly used lubricating oils, whether naturally occurring or synthetic and improve the 25 penetrating power of such oils. It has been found that the penetrating qualities of the lubricating oil bases are enhanced to a desirable degree with from 1.0% to 5.0% by volume, based on the total volume of the composition, of the compounds described above. A preferred range 30 is from 2.0 to 4.0 volume per cent of the acetals or mercaptals. Especially preferred are blends of from 2.0 to 4.0 volume per cent of an acetal or mercapta in an aromatic base stock.

35 The effectiveness of penetrating oils is often measured by the spreading rate, or the time required to penetrate a standard sintered cup, or a series of sintered cups. This rate of penetration is considered significant when such equipment as rusty bolts, nuts, hinges, and farm 40 machinery are being lubricated. Increased penetrating power is also desirable in other more general lubricating problems, such as the oiling of springs on automobiles, trucks, wagons, and the like.

45 Examples of the instant invention are tabulated below. The time required for the first drop of the penetrating composition to pass through a series of four sintered cups is used as an indication of penetrating ability.

50 Base stocks for penetrating oils are desirably aromatic because of the greater penetrating properties of aromatic compounds. The components of preferable base stocks are described below:

55 Base A.—Mixture of hydrocarbons containing at least 95% aromatic monocyclic compounds. Among the compounds are trimethyl benzene, propyl benzene, etc. Boiling point 310° to 345° F.

60 Base B.—An aromatic extract from virgin kerosene containing approximately 80% aromatics. Boiling point 300 to 530° F.

65 Base C.—Fraction from cycle gas stock obtained from catalytic cracking units. It has approximately 80% aromatics and a boiling point of 380° to 500° F.

Base D.—Light neutral oil distillate from naphthenic crude. It has a viscosity at 210° F. of 37 SUS.

65 In accordance with the concept of the instant invention a series of blends were prepared by admixing 3.0 volume percent of various acetals and mercaptals as described above with 97.0 volume percent of a base stock 70 which was composed of 40.0 volume percent of base A, 30.0 volume percent of base C, and 30.0 volume percent of base D. The blends were then submitted to the

standard sintered crucible test as described above. Resulting data are set out below:

Table I

| Acetal                                                               | Time in seconds for first drop of oil to pass through 4 sintered cups at 68° F. |
|----------------------------------------------------------------------|---------------------------------------------------------------------------------|
| Base stock                                                           | 190                                                                             |
| Di-isodecyl acetal of C <sub>8</sub> oxo aldehyde                    | 182                                                                             |
| Di-isotridecyl mercaptal <sup>1</sup> of C <sub>8</sub> oxo aldehyde | 178                                                                             |
| Di-isooctyl acetal of C <sub>8</sub> oxo aldehyde                    | 178                                                                             |
| Di-n butyl acetal of nonylaldehyde                                   | 165                                                                             |

<sup>1</sup> Isotridecyl mercaptal used in the mercaptal was obtained from isodecyl alcohol which had been produced from UOP C<sub>12</sub> olefin by oxonation.

It will be noted that the acetals and mercaptals markedly improve the penetrating power of the base stock blend.

In a second series of experiments a base stock blend of 40.0 volume percent of base B, 30.0 volume percent of base C and 30.0 volume percent of base D was used. Various acetals prepared in accordance with the above description were blended with this base stock and the standard penetration test performed. Data on this series of experiments are recorded in Table II below.

Table II

| Acetal                                                         | Time in seconds for first drop of oil to pass through 4 sintered cups at 68° F. |
|----------------------------------------------------------------|---------------------------------------------------------------------------------|
| Base stock                                                     | 203                                                                             |
| Di-n-butyl acetal of nonylaldehyde <sup>1</sup>                | 190                                                                             |
| Di-isooctyl acetal of C <sub>8</sub> oxo aldehyde <sup>2</sup> | 187                                                                             |
| Di-isodecyl acetal <sup>3</sup> of C <sub>8</sub> oxo aldehyde | 186                                                                             |
| Di-n-decyl acetal of C <sub>8</sub> oxo aldehyde               | 186                                                                             |

<sup>1</sup> Nonyl aldehyde obtained by oxonation of diisobutylene.

<sup>2</sup> Isooctyl alcohol and C<sub>8</sub> oxo aldehyde derived from propylene-butylene codimer by oxonation.

<sup>3</sup> Isodecyl alcohol used in the acetal was obtained by oxonation of tripropylene.

The data reported above will show the marked improvement in penetrating power obtained by the compositions in accordance with this invention.

To summarize briefly, the instant invention relates to improved penetrating oils which comprise a blend of a hydrocarbon oil, preferably an aromatic base stock with from 1.0 to 5.0% by volume of a material formula:



wherein R is an aliphatic radical derived from an aldehyde and containing from 4 to 18 carbon atoms, preferably 7-12 carbon atoms, wherein R is an alkyl radical derived from an alcohol or a mercaptan and containing from 4 to 18 carbon atoms, preferably 7-12 carbon atoms, and wherein X is oxygen or sulfur.

What is claimed is:

1. An improved penetrating oil which comprises a mineral oil base stock containing combined therein a minor amount, sufficient to improve the penetrating power thereof, of a material having the formula: RCH(XR')<sub>2</sub> wherein R and R' are alkyl radicals having from 4 to 18 carbon atoms and wherein X is selected from the class of oxygen and sulfur.

15 2. An improved penetrating oil which comprises a mineral oil base stock containing combined therein a minor amount, but sufficient to improve the penetrating power thereof, of an acetal of the formula: RCH(OR')<sub>2</sub> wherein R and R' are alkyl radicals containing from 4 to 18 carbon atoms.

20 3. An improved penetrating oil composition which comprises a mineral oil base stock containing combined therein a minor amount, but sufficient to improve the penetrating power thereof of a material of the formula: RCH(SR')<sub>2</sub> wherein R and R' are alkyl radicals containing from 4 to 18 carbon atoms.

25 4. A penetrating oil composition according to claim 1 wherein R and R' contain from 7 to 12 carbon atoms each.

5 5. An improved penetrating oil composition which comprises a highly aromatic mineral oil base stock containing combined therein from 1.0% to 5.0% by volume, based on the volume of the total composition, of a material of the formula: RCH(XR')<sub>2</sub> wherein R and R' are alkyl radicals containing from 7 to 12 carbon atoms and wherein X is selected from the group of oxygen and sulfur.

6. An improved penetrating oil composition according to claim 5 wherein X is oxygen.

7. An improved penetrating oil composition according to claim 5 wherein X is sulfur.

40 8. An improved penetrating oil composition which comprises a blend of highly aromatic mineral oil basis containing combined therein from 2.0 to 4.0 vol. percent, based on the volume of the total composition of the di-n-butyl acetal of nonyl aldehyde.

45 References Cited in the file of this patent  
UNITED STATES PATENTS

- |           |          |       |               |
|-----------|----------|-------|---------------|
| 2,321,593 | Gresham  | ----- | June 15, 1943 |
| 2,446,944 | Morgan   | ----- | Aug. 10, 1948 |
| 2,448,093 | Gittings | ----- | Aug. 31, 1948 |
| 2,512,771 | Glavis   | ----- | June 27, 1950 |
| 2,668,862 | Price    | ----- | Feb. 9, 1954  |